

## UNITED STATES PATENT OFFICE

2,085,903

## PRODUCTION OF MEDIUM-TEMPERATURE COKE

Wilhelm Fitz, Essen, Germany, assignor, by mesne assignments, to Koppers Company, a corporation of Delaware

No Drawing. Application January 19, 1934, Serial No. 707,419. In Germany January 20, 1933

1 Claim. (Cl. 202—20)

My invention relates to the carbonization of fuel, such as finely divided and well coking coal, especially bituminous coal and the like, and has particular reference to the so-called medium 5 temperature carbonization of fuels, that is, a carbonization process which is carried through in such a manner that no portion of the coke produced, when gradually reheated in a closed space, for instance in a closed electric furnace, 10 begins to give off gas outside the range of temperature of from 600 to 750° centigrade.

The temperature at which gases begin to escape from coke being slowly reheated in an air-tight oven is determined in the usual manner by tracing 15 the tangent on that section of the curve of carbonization, which shows uniform formation of gases. By "curve of carbonization" I mean a curve which indicates the quantity of gas delivered at different temperatures by a determined 20 quantity of coke when gradually heated. In order to facilitate comprehension, it may be mentioned that the usual high temperature coke or blast furnace coke begins to give off gases at temperatures of from 700 to 830° centigrade or 25 more.

In the medium temperature carbonization the coal is heated preferably in a chamber coke oven made of a suitable ceramic material, such as fire-clay bricks, to a temperature of about 600— 30 750° centigrade, the walls of the coking chamber being kept at a temperature, measured on the inner side of the chamber wall, which does not exceed the aforesaid temperature. The coke is withdrawn from the coking chamber as soon as 35 the condensable hydrocarbons cease to escape from the coking charge. In the medium temperature carbonization an easily inflammable and reactive coke in large solid pieces is obtained which burns without smoke and as to its properties of 40 combustion closely resembles the natural anthracite or semi-anthracite. In addition, by-products are obtained which practically have the same market value as the known by-products of the high temperature carbonization. In this 45 latter respect the medium temperature carbonization process is superior to the known low temperature carbonization which preferably is carried out in iron retorts or the like.

The object of my invention is to provide improvements in the medium temperature carbonization of fuels, especially finely divided well coking coal of all sorts, in such a manner, that the carbonization process proper can be carried through within a shorter time and thus notably 50 more economically than it was hitherto possible.

In order to produce medium temperature coke in an economically still admissible relatively short coking time, the mass to be carbonized must have the best possible heat conductivity and the consumption of heat required for the carbonization 55

must be as small as possible. Furthermore, the material to be subjected to the medium temperature coking process must show, already at the coking temperatures above indicated of the medium temperature carbonization, such a contraction, that it can be removed from the coking chamber without difficulty, for example with the known horizontal chamber ovens by means of the usual pushers. With most of the well coking coal sorts both these conditions are improved to the 10 desired extent by adding finely divided coal which has been subjected to a preliminary heat treatment at temperatures below its softening point, or finely divided coal particles obtained by the dry heating of coal to temperatures slightly 15 above the softening point (low temperature coke).

The above additions when compared with crude coal, possess a comparatively high heat conductivity. Consequently, mixtures of crude coal and the above indicated additions require a 20 notably shorter coking time than pure crude coal. Besides, the contraction of the coal and thus of the product of the carbonization is improved by the additions indicated to such an extent, that practically no difficulties arise in pushing from 25 the coking chamber medium temperature coke obtained by coking a mixture of crude coal and the above additions.

Hitherto the mixture of crude coal and one of the above-named additions has been subjected to the medium temperature carbonization in cold state. With a width of the coking chamber of about 350 mm. the carbonization time amounts to about 24 hours. This time, however, is very long, considering the comparatively high costs 30 of the medium temperature carbonization plants, that means, the output of the coking plant is very small with relation to the invested funds, to obtain a satisfying lucrative coking process.

Now, according to my present invention, in order to accelerate the coking process proper of the medium temperature carbonization process and thus to improve the economy of the process, the mixture of finely divided, well-coking crude coal and an addition of the kind indicated above 40 is previously to being filled into the coking chamber, preheated and that to temperatures lying below that point at which the mixture softens or cakes together, and thereupon is charged in such preheated state into the coking chamber.

It has already been suggested to preheat to 50 temperatures below the softening point, previous to the carbonization, a badly coking coal that is to be subjected to high temperature carbonization. These proposals, however, never have been 55 realized successfully, as tests have shown that no advantage is obtained in the high temperature carbonization by such preheating treatment. Besides, high temperature coke made from a preheated, badly coking coal is of a notably lower 60

quality than coke made from crude coal charged in cold and wet state. This results from the feature which frequently is overlooked, viz., that the badly coking coal sorts, when preheated even 5 in an hermetically closed space, more or less lose their coking capacity which already is small in itself. On the other hand, when finely disintegrated cold crude coal with a moisture of more than about 10% is used, the coal enters the coking chamber in the state of highest baking capacity and, owing to the comparatively high percentage of moisture, it is maintained at a low temperature for a rather long time during the carbonization, so that also the preheating period 10 of the coal during the carbonization process is remarkably shortened, and consequently, those alterations of the substance of the coal cannot occur at all or to a very small extent only, which unfavourably influence its coking capacity.

20 In contrast thereto, I have discovered by my tests, that well-coking coals, that is, coals rich in bright coal, which coke very well and have a high content of binding substances, can be preheated for a considerably longer period of time, without 25 affecting the original baking capacity seriously. Such well coking coals, however, are preferably used in the medium temperature carbonization, as they possess the capacity of binding in a sufficient quantity of the above indicated additions, 30 which are required for the economical carrying out of the medium temperature carbonization.

I obtain very important advantages unknown 35 hitherto by preheating the material to be charged in the medium temperature carbonization: In the first place the consumption of heat required for the formation of coke is considerably reduced. Furthermore, the preheated mixture of crude coal and an addition of the above kind has a notably 40 higher heat conductivity, since semi-coke has a positive coefficient of heat conductivity, that means, the heat conductivity of semi-coke increased with increasing temperature. All these features result, in the execution of the process according to my invention, in a notably shortened 45 carbonization time, without any perceptible noxious influence being exerted on the quality of the produced coke by the preheating of the mixture to be coked.

Thus the economy of the medium temperature 50 carbonization is substantially improved by the process according to my invention.

A further advantageous effect of my invention resides in the fact, that it is now possible, under 55 certain circumstances, to carry through the medium temperature carbonization in the usual coking chambers of a width of more than 350 mm., without the carbonization time needing to be prolonged to such an extent, that the coke gives off gases to a large extent in the marginal 60 layers, that is, up to the extent to be observed in the high temperature carbonization. Consequently, the application of my process also secures in coking chambers of greater width the production of a technically homogeneous medium temperature coke of good quality. The somewhat 65 longer carbonization time can be tolerated in most cases of existing coking plants with wider coking chambers without disadvantage, since these older plants as a rule already have been deemed completely, so that the coke is not required 70 to carry the interest on the invested capital.

My improved coking process is carried through in practice for example in the following manner:

75 A mixture composed of crude coking coal and

the addition, for example semi-coke, and containing about from 55 to 60% well coking coal and further a small percentage of small coke as it remains in the disintegration of the medium temperature coke, is preheated, preferably in a 5 hermetically sealed container, to a temperature of the softening point of the coal or to that point at which the mixture cakes together. The temperature to which the mixture of coal and semi-coke is to be preheated, depends upon the properties of the coal to be treated. As preheating devices I use with advantage the usual rotary drum furnaces with direct or better indirect heating appliance. From these rotary drum furnaces the preheated mixture then is conveyed to an 15 intermediate bunker of a small size. From there the heated mass after a short time without coming into contact with air is delivered into the larry car which advantageously is insulated, and then charged into the coking chamber. Where 20 horizontal chamber ovens are used for the execution of my coking process, the mixture is charged preferably through one sole charging hole disposed in the midst of the coking chamber, since the dry mixture is distributed uniformly 25 on the chamber almost without any outer help.

According to the composition of the mixture and to the temperature obtainable in the preheating treatment the carbonization time is reduced about to half that required for medium 30 temperature carbonization without preheating treatment of the mixture. In other words, for the same output the plant can be designed half as great as and thus at lower costs, than hitherto. Finally, the preheating treatment affords the advantage that a better and more uniform medium 35 temperature coke is obtained.

I wish it to be understood that the preceding 40 specification describes only an example of one way of carrying out my invention which, however, is not confined to this example. On the contrary, various modifications may be provided in the process above described, without in any way departing from the spirit of the invention as defined in the appended claim, and the right to 45 make subsequent claims other than the following is expressly reserved.

What I claim is:—

A method of making medium temperature coke by which the coking period is reduced about one 50 half from well coking finely divided bituminous coal and similarly caking carbonizable fuel in a coking chamber consisting of ceramic material heated by externally applied heat which process 55 comprises: separately preliminarily preheating a mixture consisting of about 55% to 60% of well coking coal rich in bright coal and having a high content of binding substances and low temperature coke, prior to introducing the mixture into the coking chamber, up to a temperature approximating but lying below that point at which the mixture softens and cakes together; charging the mixture in such preheated condition into the coking chamber and coking the same therein separately from the preheating by externally applying heat to the walls of the coking chamber to a maximum temperature of from 600° to 750° centigrade, measured on the inner side of the chamber wall, throughout the carbonization to 60 effect and complete the carbonization; and withdrawing the coke formed as soon as condensable hydrocarbons cease to escape from the coking mixture.